

# United States Patent

Iwama et al.

[15] 3,649,285

[45] Mar. 14, 1972

[54] **LIGHT-SENSITIVE SILVER HALIDE COLOR PHOTOGRAPHIC MATERIALS CONTAINING CYAN COUPLER**

[72] Inventors: **Masakuni Iwama; Toshihiko Yamamoto; Keiji Kasai; Yoshinobu Nakagawa; Takaya Endo, all of Tokyo, Japan**

[73] Assignee: **Konishiroku Photo Industry Co., Ltd.**

[22] Filed: **July 13, 1970**

[21] Appl. No.: **54,625**

[30] **Foreign Application Priority Data**

July 16, 1969 Japan.....44/55733

[52] U.S. Cl.....96/100, 96/9

[51] Int. Cl.....G03c 1/40

[58] Field of Search.....96/55, 100

[56] **References Cited**

UNITED STATES PATENTS

|           |         |                 |             |
|-----------|---------|-----------------|-------------|
| 2,186,850 | 1/1940  | Wilmanns et al. | .....96/100 |
| 2,476,559 | 7/1949  | Nawiasky et al. | .....96/100 |
| 2,860,974 | 11/1958 | Williams        | .....96/100 |
| 3,271,152 | 9/1966  | Hanson          | .....96/100 |

Primary Examiner—J. Travis Brown

Attorney—Harry C. Bierman, Jordan B. Bierman and Bierman & Bierman

[57]

## ABSTRACT

A coupler having the formula



wherein R is an aryl or aralkyl group or unsaturated aliphatic hydrocarbon residue having one to 22 carbon atoms, R' is an aliphatic residue having one to six carbon atoms, and X is hydrogen or halogen is incorporated within a light-sensitive silver halide color photographic emulsion. A composition useful for forming a cyan-colored photographic image is produced. Deposition of the coupler in the emulsion is substantially reduced. The color formation rate of the coupler is close to that of other magenta and yellow couplers. This enables the three colors to be readily balanced in speed. A finely grained color image is obtained upon color development.

2 Claims, No Drawings

**LIGHT-SENSITIVE SILVER HALIDE COLOR  
PHOTOGRAPHIC MATERIALS CONTAINING CYAN  
COUPLER**

The present invention relates to a light-sensitive color photographic material incorporated with a novel coupler for forming a cyan-colored photographic image.

For the formation of a color photographic image according to the conventional subtractive color photography, there have been used, in general, couplers capable of coupling with an oxide of the N,N-disubstituted p-phenylene-diamine-type developing agent to form yellow, cyan and magenta colors. Particularly in the case of the so-called internal color photography in which said couplers are incorporated into photographic emulsions to form the colors, there are two processes; a process in which water-solubilizing groups (e.g.,  $\text{SO}_3\text{H}$  and  $\text{COOH}$  groups) are introduced into the molecules of the couplers, the thus treated couplers are dissolved in alkali solution or the like and the resulting solutions are added to the emulsions, and a process in which the couplers are made oil-soluble by introducing oil-solubilizing groups (e.g., higher alkyl groups) into the molecules thereof and dissolved in various organic solvents (e.g., di-n-butyl phthalate and the like), and the resulting solutions are added to the emulsions.

It is needless to say that color images obtained by color development are desired to be favorable in color reproducibility, excellent in color tone and high in stability to light, heat and temperature. In this respect, it has been said to be desirable to use so-called protect-type couplers which are water-insoluble or difficultly water-soluble and which can be dissolved in organic solvents and dispersed in photographic emulsions. Particularly important conditions in the case where said protect-type couplers are used are such that the couplers should have sufficient solubilities for organic solvents (hereinafter referred to as "coupler solvents"), and should not deposit or agglomerate even when dispersed in photographic emulsions and even after coated as light-sensitive materials on supports. In view of the above, many oleophilic components have chiefly been examined and studies on the synthesis of various derivatives have been made. However, most of the couplers obtained do not show sufficient solubilities for the coupler solvents, or are insufficient in dispersibility in photographic emulsions and deposit when added to the emulsions or after being coated on supports. Further, cyan couplers are higher, in general, in color formation rate than magenta and yellow couplers, and therefore the resulting color images are not well balanced in density, in most cases. In order to make the balance in density of color image more favorable, there have been made many such attempts that the speed of red-sensitive layer is decreased or the speeds of green- and blue-sensitive layers are increased.

An object of the present invention is to provide a light-sensitive photographic material incorporated with a cyan coupler, which shows sufficient solubility for a coupler solvent, e.g., di-n-butyl phthalate, o-tricresyl phosphate, di-n-butyl lauramide or ethyl acetate and which does not deposit or agglomerate after the coupler dispersion has been dispersed in a photographic emulsion or after the coupler-incorporated emulsion has been coated on a support.

Another object of the invention is to provide a novel coupler, which can inhibit the color formation rate of naphthol-type cyan coupler to obtain the balance of 3 layers and, at the same time, can have a dye formed in fine grain state by color development.

Conventional cyan couplers, e.g., 1-hydroxy-2-naphthamide type derivatives of the formula,



wherein R is a higher alkyl group, and X is a hydrogen or halogen atom, are excellent in formation efficiency of in-

doaniline dye images obtained by coupling with oxidation products of N,N'-disubstituted p-phenylenediamine type developing agents, and have excellent color tones. However, the conventional couplers have many such practical drawbacks that they are inferior in solubility for coupler solvents and severely deposit in photographic emulsions, and most of the particles of the formed dyes are coarse.

As an attempt to increase the solubility for coupler solvents, Japanese Pat. Publication No. 11,303/1967 proposes the use of couplers represented by the formula (II) in which has been formed such an oxazine ring as shown below.



20  
25  
wherein R is a saturated hydrocarbon, and X is a hydrogen or halogen atom.

30  
35  
However, the couplers of this kind are extremely low in coupling rate at the time of color development and hence are substantially impractical, though they have somewhat been improved in solubility.

In view of the above, we have made various studies to find couplers represented by the general formula (III) shown below which are free from such drawbacks as seen in the couplers of the general formulas (I) and (II) and which can sufficiently satisfy the objects of the present invention.



45  
50  
wherein R is a substituted aryl or aralkyl group or a saturated or unsaturated and substituted or unsubstituted aliphatic hydrocarbon residue having one to 22 carbon atoms; R' is an aliphatic hydrocarbon residue having one to six carbon atoms; and X is a hydrogen or halogen atom.

55  
60  
65  
70  
The alkoxalyl-type cyan couplers represented by the above-mentioned general formula have increased solubilities for coupler solvents. Particularly, those of the said general formula (III), in which R' is an aliphatic hydrocarbon residue having four to six carbon atoms, could be easily dissolved in coupler solvents of one-half to one-third of the amounts required in the case of corresponding couplers represented by the general formula (I), and, even when the solutions were allowed to stand at room temperature, they were extremely long in time required for initiation of deposition. Further, they showed improved oil solubilities. The solubility test was carried out in such a manner that 1 g. of a coupler of the present invention was dissolved in di-n-butyl phthalate over a water bath at 60° C., and the resulting solution was allowed to stand at 20° C. to observe the crystallization initiation time of the coupler. The properties of corresponding couplers of the general formula (I) were also measured at the same time and compared with those of the present couplers. The present couplers in which R'=C<sub>2</sub> were substantially identical in solubility with the couplers of the general formula (I), but those in which R'=C<sub>4</sub> H<sub>9</sub> were considerably improved both in solubility and in deposition characteristic, as shown in the following table.

|                                                                                      | Control coupler |                                                                                                                         | Present coupler           |                            |                           |                            |
|--------------------------------------------------------------------------------------|-----------------|-------------------------------------------------------------------------------------------------------------------------|---------------------------|----------------------------|---------------------------|----------------------------|
|                                                                                      | R=H             | R=  -O-C <sub>4</sub> H <sub>9</sub> | Amount of coupler solvent | Deposition initiation time | Amount of coupler solvent | Deposition initiation time |
|  OR |                 |                                                                                                                         | 10 ml.....                | 5 hrs.....                 | 5 ml.....                 | 7 hrs.                     |
|  OR |                 |                                                                                                                         | 1 ml.....                 | No deposition...           | 1 ml.....                 | No deposition.             |
|  OR |                 |                                                                                                                         | 5 ml.....                 | 5 hrs.....                 | 5 ml.....                 | No deposition.             |
|  OR |                 |                                                                                                                         | 10 ml.....                | 60 min.....                | 5 ml.....                 | 20 hrs.                    |

As seen in the above table, the couplers prepared by changing the hydroxyl groups of the couplers of the general formula (I) to



are increased in solubility for coupler solvents to make it possible to obtain coupler solutions of high concentration. 45 Even when these solutions are allowed to stand, the crystallization of the couplers is extremely slow.

Further, when the photographic emulsion having the present coupler dispersed therein is coated on a support, the amount of high boiling solvent per unit area is small, and therefore the emulsion is less affected by the high boiling solvent and can be easily formed into a thin layer to give such advantage that the resulting color image is improved in sharpness.

The present coupler of the general formula (III) is 55 somewhat lower in color formation rate than a corresponding coupler of the general formula (I). This, however, results in such advantage that the coupler becomes close in color formation rate to other magenta and yellow couplers, with the result that the 3 colors can easily be balanced in speed.

Further, in the case of the present coupler, the dye formed by color development becomes finer in grain size than in the case of a corresponding coupler of the general formula (I) to make it possible to obtain a color image with extremely fine grains.

In addition to the above-mentioned advantages, the coupler of the present invention has such important significance as set forth below.

That is, even when the OH group in the 1-position is changed to such an alkoxaloyloxy group as seen in the general formula (III), the coupler is not hindered in function and, moreover, the alkoxaloyl group in the 1-position is removed during the step of color development to form the same dye as that formed from a corresponding coupler of the general formula (I), as shown below, for example.



Examples of the coupler compounds represented by the general Formula (III) which are used in the present invention are as shown below, but these are, of course, not limitative.

(1)



(2)





Further, as R in the general formula (III), there may be introduced any of the following groups:



wherein n is an integer of 1 to 6.

These compounds can easily be synthesized by reacting corresponding 1-hydroxy-2-naphthamide type couplers with alkoxaryl chlorides in xylene or acetonitrile.

Synthesis examples of typical couplers are set forth below.

Synthesis Example II

Synthesis of ethoxalyl chloride

75 25.3 g. of oxalyl chloride was charged into a three-necked

flask. Into this was dropped with stirring 9.2 g. of ethanol over a period of 1 hour while maintaining the inner temperature at below 10° C. The resulting mixture was reacted with stirring at room temperature for 30 minutes and then subjected to distillation to obtain 18.3 g. of ethoxalyl chloride, yield 69 percent, b.p. 134°-136° C.,  $n_D^{20}$  1.4170.

#### Synthesis Example II

##### Synthesis of butoxalyl chloride

Synthesis Example I was repeated, except that 6.8 g. of *n*-butanol was used in place of the ethanol, to obtain 10.3 g. of a colorless liquid, yield 68 percent, b.p. 73°-75° C./8 mm.Hg.,  $n_D^{20}$  1.4252.

#### Synthesis Example III

##### Synthesis of 1-ethoxalyoxy-N-[w-(2,4-di-tert-arylphenoxy) butyl]-2-naphthamide (Exemplified compound 6):

A mixture comprising 4.7 g. of 1-hydroxy-N-[w-(2,4-di-tert-arylphenoxy) butyl]-2-naphthamide, 25 ml. of pyridine and 15 ml. of acetonitrile was charged into a 50 ml. three-necked flask. To the flask were attached a stirrer, a thermometer and a dropping funnel. Further, a calcium chloride tube was attached for desiccation. Into the flask was dropped 2.6 g. of ethoxalyl chloride over a period of 40 minutes, while maintaining the inner temperature at 5° C.  $\pm$  2° C. After stirring the resulting mixture at below 10° C. for 1 hour and at room temperature for additional 1 hour, the pyridine and acetonitrile were removed by means of an aspirator, and the residue was poured into 150 ml. of ice water. The resulting pale yellow oil was extracted from 100 ml. of ethyl acetate, washed with water and then concentrated under reduced pressure. The concentrate was recrystallized from 50 ml. of *n*-hexane to obtain 3.0 g. of white sand-like crystals, yield 54.5 percent, m.p. 123°-124° C.

#### Synthesis Example IV

##### Synthesis of 1-ethoxalyoxy-N-[w-(2,4-di-tert-arylphenoxy) butyl]-4-chloro-2-naphthamide (Exemplified compound 13):

1-Hydroxy-N-[w-(2,4-di-tert-arylphenoxy) butyl]-4-chloro-2-naphthamide was treated in the same manner as in Synthesis Example III to obtain white sand-like crystals, yield 55 percent, m.p. 122°-123° C.

#### Synthesis Example V

##### Synthesis of 1-butoxalyoxy-N-[w-(2,4-di-tert-arylphenoxy) butyl]-2-naphthamide (Exemplified compound 7):

Synthesis Example III was repeated, except that *n*-butoxalyl chloride was used in place of the ethoxalyl chloride, to obtain white sand-like crystals, yield 55 percent m.p. 96°-97° C.

#### Synthesis Example VI

##### Synthesis of 1-ethoxalyoxy-N-(n-dodecyl)-2-naphthamide (Exemplified compound 1):

A mixture comprising 3.6 g. of N-n-dodecyl-1-hydroxy-2-naphthamide, 25 ml. of pyridine and 15 ml. of acetonitrile was charged into a 50 ml. three-necked flask. To the flask were attached a stirrer, a thermometer and a dropping funnel. Further, a calcium chloride tube was attached for desiccation. The inner temperature of the flask was lowered to 5° C.  $\pm$  2° C., while stirring the mixture. Into the flask was dropped 2.7 g. of the ethoxalyl chloride synthesized in Synthesis Example I over a period of 40 minutes. After the dropping, the mixture

was stirred at below 20° C. for 1 hour and at room temperature for additional 1 hour. Subsequently, the pyridine and acetonitrile were removed by means of an aspirator, and the residue was poured into 150 ml. of ice water to precipitate a pale yellow oil. The oil was extracted from 100 ml. of ethyl acetate, washed with water and concentrated under reduced pressure. The concentrate was recrystallized from 50 ml. of *n*-hexane to obtain 2.5 g. of white needlelike crystals, yield 56 percent, m.p. 98°-99° C. According to infrared analysis, the

crystals showed characteristic absorptions at 1,760 cm.<sup>-1</sup> and 1,650 cm.<sup>-1</sup>.

#### Synthesis Example VII

##### Synthesis of 1-ethoxalyoxy-N-(n-dodecyl)-4-chloro-2-naphthamide (Exemplified compound 8):

15 N-n-dodecyl-1-hydroxy-4-chloro-2-naphthamide was treated in the same manner as in Synthesis Example VI to obtain white needlelike crystals, yield 72 percent, m.p. 97°-98° C.

#### Synthesis Example VIII

##### Synthesis of 1-butoxalyoxy-N-(n-dodecyl)-4-chloro-2-naphthamide (Exemplified compound 9):

Synthesis Example VI was repeated, except that butoxalyl chloride and N-n-dodecyl-1-hydroxy-4-chloro-2-naphthamide were used in place of the ethoxalyl chloride and N-n-dodecyl-1-hydroxy-2-naphthamide, to obtain white needlelike crystals, yield 88 percent, m.p. 88°-89° C.

#### Synthesis Example IX

##### Synthesis of 1-ethoxalyoxy-N-n-dodecyl-4-iodo-2-naphthamide (Exemplified compound 10):

Synthesis Example VI was repeated, except that N-n-dodecyl-1-hydroxy-4-iodo-2-naphthamide was used in place of the N-n-dodecyl-1-hydroxy-2-naphthamide, to obtain white needlelike crystals, yield 69.0 percent, m.p. 68°-69° C.

#### Synthesis Example X

##### Synthesis of 1-ethoxalyoxy-N-(n-octadecyl)-2-naphthamide (Exemplified compound 3):

Synthesis Example VI was repeated, except that N-n-octadecyl-1-hydroxy-2-naphthamide and xylene were used in place of the N-n-dodecyl-1-hydroxy-2-naphthamide and acetonitrile, to obtain white needlelike crystals, yield 85 percent, m.p. 99°-100° C.

#### Synthesis Example XI

##### Synthesis of 1-ethoxalyoxy-N-(octadecenyl)-2-naphthamide (Exemplified compound 5):

A mixture comprising 4.3 g. of N-octadecenyl-1-hydroxy-2-naphthamide, 13 ml. of pyridine and 15 ml. of acetonitrile was charged into a 50 ml. three-necked flask. To the flask were attached a stirrer, a thermometer and a dropping funnel. Further, a calcium chloride tube was attached for desiccation. The inner temperature of the flask was maintained at 5° C.  $\pm$  2° C., and 2.7 g. of ethoxalyl chloride was gradually dropped into the flask with stirring. Thereafter, the same operation as in Synthesis Example VI was effected to obtain 3.6 of a butter-like oily substance, yield 67 percent. According to infrared analysis, the thus obtained substance showed a characteristic absorption at 1,750 cm.<sup>-1</sup>.

Melting points and elementary analysis values of typical couplers used in the present invention are shown in Table 1.

TABLE 1

Elementary analysis values

| Exemplified compound | M.p. (° C.) | Calculated |      |      | Found      |       |      |      |            |
|----------------------|-------------|------------|------|------|------------|-------|------|------|------------|
|                      |             | C          | H    | N    | Cl         | C     | H    | N    | Cl         |
| 1                    | 98~99       | 71.18      | 8.19 | 3.07 | .....      | 71.11 | 8.31 | 3.10 | .....      |
| 2                    | 98~99       | 72.76      | 8.86 | 2.74 | .....      | 72.68 | 8.89 | 2.79 | .....      |
| 3                    | 99~100      | 73.43      | 9.18 | 2.60 | .....      | 73.18 | 9.42 | 2.88 | .....      |
| 4                    | 86~7        | 74.03      | 9.41 | 2.47 | .....      | 74.12 | 9.63 | 2.56 | .....      |
| 5                    | (*)         | 73.71      | 8.81 | 2.61 | .....      | 73.48 | 8.82 | 2.97 | .....      |
| 6                    | 123~4       | 73.01      | 7.88 | 2.43 | .....      | 72.71 | 7.91 | 2.59 | .....      |
| 7                    | 96~7        | 73.60      | 8.18 | 2.32 | .....      | 73.22 | 8.31 | 2.72 | .....      |
| 8                    | 97~8        | 66.17      | 7.41 | 2.86 | 7.23       | 66.47 | 7.62 | 2.88 | 7.16       |
| 9                    | 88~9        | 67.23      | 7.78 | 2.70 | 6.84       | 67.08 | 7.88 | 2.88 | 6.75       |
| 10                   | 68~9        | 55.77      | 6.24 | 2.42 | 21.83 (I)  | 55.50 | 6.16 | 2.30 | 21.65 (I)  |
| 11                   | 92~3        | 68.17      | 8.12 | 2.56 | 6.49       | 68.10 | 8.32 | 2.43 | 6.41       |
| 12                   | 86~7        | 69.03      | 8.43 | 2.44 | 6.17       | 68.91 | 8.51 | 2.32 | 6.28       |
| 13                   | (*)         | 69.27      | 8.10 | 2.45 | 6.20       | 69.21 | 8.05 | 2.33 | 6.45       |
| 14                   | 122~3       | 68.89      | 7.27 | 2.29 | 5.81       | 68.78 | 7.25 | 2.65 | 5.65       |
| 15                   | 168~72      | 66.12      | 4.93 | 2.86 | 16.30 (Br) | 66.01 | 4.99 | 3.02 | 16.04 (Br) |
| 16                   | 168~174     | 74.04      | 6.57 | 2.46 | .....      | 74.16 | 6.33 | 2.72 | .....      |

The present invention is illustrated in further detail below with reference to examples, but the examples are illustrative, and it is needless to say that the invention is not limited thereto.

### EXAMPLE 1

10 g. of the exemplified coupler compound 4 was completely dissolved at 60° C. in a mixed liquid comprising 10 ml. of di-n-butyl phthalate and 20 ml. of ethyl acetate. This solution was mixed with 10 ml. of a 10 percent aqueous solution of Alkanol B (trade name of Du Pont) and 200 ml. of a 5 percent aqueous gelatine solution, and the resulting mixture was subjected to a colloid mill to form a dispersion. The dispersion was added to 1,000 ml. of a red-sensitive silver iodobromide photographic emulsion, which was then coated on a film base, followed by drying, to obtain a light-sensitive color photographic material.

The thus obtained film was exposed and then developed at 20° C. for 10 minutes with a developer of the following composition:

|                                              |           |
|----------------------------------------------|-----------|
| N,N-Diethyl-p-phenylenediamine hydrochloride | 2.0 g.    |
| Anhydrous sodium sulfite                     | 2.0 g.    |
| Sodium carbonate (monohydrate)               | 82.0 g.   |
| Potassium bromide                            | 2.0 g.    |
| Water to make                                | 1,000 ml. |

Subsequently, the film was subjected to stopping and fixing according to ordinary procedures, washed with water for 10 to 15 minutes and then treated for 5 minutes with a bleaching solution of the following composition:

|                   |           |
|-------------------|-----------|
| Red prussiate     | 100 g.    |
| Potassium bromide | 50 g.     |
| Water to make     | 1,000 ml. |

The film was further washed with water for 5 minutes and then fixed for 5 minutes with the following fixing bath:

Sodium thiosulfate (pentahydrate) 250 g.  
Water to make 1,000 ml.

Thereafter, the film was washed with water and then dried. The thus treated film was excellent in transparency and had a cyan color image of fine grains having an absorption maximum at  $690\text{ }\mu$ .

Photographic properties of films obtained in the same manner as in Example 1, except that in place of the exemplified compound 4, there were used either singly or in combination the compounds A and B shown below which corresponded to the general formulas (I) and (III), respectively, are as shown in Table 2.



| Compound      |           | Photographic properties |       |                 |                |
|---------------|-----------|-------------------------|-------|-----------------|----------------|
| A             | B         | Relative speed          | Gamma | Maximum density | Graininess     |
| 10 parts..... |           | 100                     | 0.95  | 1.86            | Coarse.        |
|               | 10 parts  | 65                      | 0.87  | 1.60            | Fine.          |
| 5 parts.....  | 5 parts.. | 90                      | 0.93  | 1.80            | Somewhat fine. |
| 2 parts....   | 8 parts.. | 80                      | 0.91  | 1.70            | Fine.          |

As is clear from Table 2, it is understood that as compared with the film prepared by use of the compound A, the film prepared by use of the present compound B is low in gamma value and the graininess of a color image obtained by printing the said film is excellent. This shows the fact that the coupler of the present invention is useful for obtaining three well-balanced layers and for improving the graininess of the resulting image. When the couplers are used in admixture, no deposition of the couplers is observed, and therefore it is possible to obtain a color image excellent in transparency. In case the coupler matrix is same, as shown in Table 2, a same dye is formed and the calculation of color balance is easy. Furthermore, such coupler is advantageously low in cost.

15 The coupler of the present invention may be used in combination with such a cyan color coupler as represented by the general formula (IV) shown below, e.g., such color coupler for obtaining a color retouching mask as exemplified in U.S. Pat. No. 3,034,892, or in combination with the couplers of the general formulas (I) and (IV), whereby the deposition characteristic of the coupler and the graininess of the resulting image 20 can be improved. The coupler of the general formula (IV) is indicated below:



wherein R and R' individually are alkyl, aryl, aralkyl or acyl group. At the same time, the coupler can be so controlled as to attain adequate masking effects. Thus, the coupler of the present invention is an extremely useful cyan coupler.

### EXAMPLE 2

40 10 g. of the exemplified coupler compound 7 was treated in the same manner as in Example 1, except that tricresyl phosphate was used in place of the di-n-butyl phthalate, to prepare a light-sensitive photographic material. After exposure, the photographic material was color-developed with the same developer as in Example 1, except that N-ethyl-N- $\beta$ -methanesulfonamide ethyl-p-phenylenediamine was used in place of the N,N-diethyl-p-phenylenediamine hydrochloride, to obtain a cyan color image of fine grains having an absorption maximum at 692  $\mu$ . Transparency of this film was quite excellent.

### EXAMPLE 3

55 15 g. of the exemplified coupler compound 1 was completely dissolved at 60° C. in a mixed liquid comprising 15 ml. of tricresyl phosphate and 45 ml. of butyl acetate. This solution was mixed with 8 ml. of a 10 percent aqueous solution of Alkanol B and 300 ml. of a 5 percent aqueous gelatine solution, and the resulting mixture was subjected to a colloid mill to form a dispersion. The dispersion was added to 1,000 ml. of a red-sensitive gelatino silver iodobromide photographic emulsion, which was then coated on a film base, followed by drying.

The thus obtained film was exposed and then developed at 20° C. for 10 minutes with a developer of the following composition:

|                               |          |
|-------------------------------|----------|
| Metol                         | 3.0 g.   |
| Anhydrous sodium sulfite      | 60.0 g.  |
| Hydroquinone                  | 6.0 g.   |
| 70 Anhydrous sodium carbonate | 50.0 g.  |
| Potassium bromide             | 1.0 g.   |
| Water to make                 | 1,000 mL |

75 Subsequently, the film was subjected to ordinary stopping and hardening treatments and water-washing. The thus treated film was further subjected to secondary exposure by

use of a white light and then developed at 20° C. for 12 minutes with a developer of the following composition:

|                                |           |
|--------------------------------|-----------|
| N,N-Diethyl-p-phenylenediamine | 5.0 g.    |
| Anhydrous sodium sulfite       | 2.0 g.    |
| Sodium carbonate (monohydrate) | 82.0 g.   |
| Potassium bromide              | 1.0 g.    |
| Water to make                  | 1,000 ml. |

The developed film was stopped, fixed, water-washed and bleached according to ordinary procedures and then washed with running water for 20 minutes, followed by drying, to obtain a positive cyan color image of fine grains having an absorption maximum at 689  $\mu$  and excellent in transparency.

## EXAMPLE 4

100 g. of the exemplified coupler compound 12 was completely dissolved at 60° C. in 100 ml. of di-n-butyl phthalate. This solution was added to 5 liters of a 10 percent aqueous gelatine solution kept at 60° C., and further charged with 200 ml. of a 10 percent aqueous sodium alkylbenzenesulfonate solution. The resulting mixture was subjected to a colloid mill at about 60° C. for 10 minutes to form a dispersion. The dispersion was stirred for 10 minutes. This operation was repeated four times with intervals of 1 minute to obtain a coupler dispersion. The thus obtained dispersion was added to 10 liters of a gelatino silver iodobromide emulsion containing a red-sensitive sensitizing dye. After thorough stirring, the emulsion was coated on a film support at 30° to 35° C. and then dried to prepare a light-sensitive color photographic material.

This film was exposed and then color-developed, bleached and fixed in the same manner as in Example 1 to obtain a cyan-colored negative image.

The film prepared by use of the exemplified coupler compound 13 was quite excellent in transparency and showed an absorption maximum at 690  $\mu$ .

40

## EXAMPLE 5

7 g. of the exemplified coupler compound 12 and 3 g. of N-n-dodecyl-1-hydroxy-4-chloro-2-naphthamide, a coupler corresponding to the general formula (I) were completely dissolved at 60° C. in a mixed liquid comprising 7 ml. of di-n-butyl phthalate and 15 ml. of ethyl acetate. This solution was mixed with 10 ml. of a 10 percent aqueous solution of Alkanol B and 200 ml. of a 5 percent aqueous gelatine solution. The resulting mixture was subjected to a colloid mill to form a dispersion. The dispersion was added to 1,000 ml. of a red-sensitive silver iodobromide emulsion, which was then coated on a film base, followed by drying to prepare a light-sensitive photographic material.

15 This film was exposed according to an ordinary procedure and then treated with the same developer as in Example 2 to obtain a cyan color image of fine grains which was excellent in transparency.

What is claimed is:

20 1. A light-sensitive silver halide color photographic emulsion incorporated with a coupler of the general formula,



wherein R is an aryl or aralkyl group or a saturated or unsaturated, aliphatic hydrocarbon residue having one to 22 carbon atoms; R' is an aliphatic hydrocarbon residue having one to six carbon atoms; and X is a hydrogen or halogen atom.

35 2. A light-sensitive silver halide color photographic element which comprises a support and, coated thereon, a light-sensitive silver halide color photographic emulsion as claimed in claim 1.

\* \* \* \* \*

45

50

55

60

65

70

75